



US006348304B1

(12) **United States Patent**  
Gula et al.

(10) **Patent No.:** US 6,348,304 B1  
(45) **Date of Patent:** Feb. 19, 2002

(54) **IMPACT RESISTANT PHOTOGRAPHIC ELEMENT**

(75) Inventors: **Thaddeus S. Gula; Richard C. McElroy**, both of Rochester; **Mamie Kam-Ng**, Fairport, all of NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/643,399**

(22) Filed: **Aug. 22, 2000**

(51) **Int. Cl.<sup>7</sup>** ..... G03C 1/79; G03C 1/93; G03C 1/765

(52) **U.S. Cl.** ..... 430/496; 430/523; 430/533; 430/534; 430/531; 430/536

(58) **Field of Search** ..... 430/536, 496, 430/534, 523, 531, 533

(56)

**References Cited**

**U.S. PATENT DOCUMENTS**

|             |        |                        |         |
|-------------|--------|------------------------|---------|
| 5,244,861 A | 9/1993 | Campbell et al. ....   | 430/201 |
| 5,888,683 A | 3/1999 | Gula et al. ....       | 430/536 |
| 5,888,714 A | 3/1999 | Bourdelaïs et al. .... | 430/536 |
| 5,935,690 A | 8/1999 | Aylward et al. ....    | 430/501 |
| 6,030,742 A | 2/2000 | Bourdelaïs et al. .... | 430/536 |

*Primary Examiner*—Richard L. Schilling

(74) *Attorney, Agent, or Firm*—Paul A. Leipold; Lynne M. Blank

(57) **ABSTRACT**

The invention relates to a photographic element comprising at least one layer of photosensitive silver halide, a base material wherein said base material comprises at least one bottom sheet of biaxially oriented polymer sheet and deformable tie layer material, wherein said deformable tie layer material yield stress of between 6 and 10 MPa in compression which is less than 10% the yield stress of any of the other layers in the element.

**11 Claims, No Drawings**

## IMPACT RESISTANT PHOTOGRAPHIC ELEMENT

### FIELD OF THE INVENTION

This invention relates to photographic materials. In the preferred form it relates to base materials for photographic prints.

### BACKGROUND OF THE INVENTION

In prior art photographic papers comprising high strength biaxially oriented polypropylene layers, great care needs to be taken in handling the materials after exposure and development of the image. Prior art silver halide photographic papers are sensitive to some compressive forces. Dot matrix printers are commonly used to conveniently add various types of useful data to the opposite side of photographic materials. If sufficient localized force is applied from the back to the opposite side photosensitive layers, permanent surface deformation of the imaging side may create undesirable disturbances to the quality of the normally smooth surface of the image. It has been found that the small diameter (250 micrometers) print heads of some dot matrix printers are accelerated at a rate to impact the printed area to cause local stresses of more than 8 MPa, these have been found to permanently deform the emulsion and imaging side components if not sufficiently cushioned. This is particularly true for special photographic materials described in U.S. Pat. Nos. 5,853,965; 5,866,282; 5,888,643; 5,888,682; 5,888,683; and 5,902,720. These photographic materials include substantial replacement of prior art typical soft, thick polyethylene layers with high modulus oriented polypropylene layers which effectively reduce the cushioning effect when printed on the backside with high pressure dot matrix printers. It would be desirable to have a photographic base material that has a degree of compressibility in a location in the element that will not affect the quality of the imaging side, thus cushioning the pressure sensitive photographic layers. This will provide a photographic base material that has increased resistance to showing the effects of localized forces that may be applied to it on the side opposite the image after exposure and development.

### PROBLEM TO BE SOLVED BY THE INVENTION

There is a continuing need for photographic base materials that have resistance to compressive load after exposure to create an image that results in fewer defects in the print after development.

### SUMMARY OF THE INVENTION

It is an object of the invention to provide photographic elements having improved resistance to concentrated backside compressive loads.

It is another object to provide photographic elements with reduced imaging side deformation caused by compressive loads after development.

It is a further object to provide photographic elements that have improved resistance to defects caused by high pressure dot matrix printers.

These and other objects of the invention are accomplished by a photographic element comprising at least one layer of photosensitive silver halide, a base material wherein said base material comprises at least one bottom sheet of biaxially oriented polymer sheet and deformable tie layer material, wherein said deformable tie layer material yield

stress of between 6 and 10 MPa in compression which is less than 10% the yield stress of any of the other layers in the element.

### ADVANTAGEOUS EFFECT OF THE INVENTION

The invention provides photographic base materials that have resistance to compressive load after exposure which results in fewer image defects in the print after development.

### DETAILED DESCRIPTION OF THE INVENTION

The invention has numerous advantages over prior practices in the art. The invention provides photographic elements that have less image side surface deformation caused by backside high pressure printing head compression during photofinishing of said elements. The flat surface will, therefore, present a pleasing image in the product without undesirable surface streaks. It will also help to reduce image discoloration caused by damage to pressure sensitive silver halide grains which results in undesirable image errors. These and other advantages will be apparent from the detailed description below.

The terms as used herein, "top", "upper", "emulsion side", and "face" mean the side or towards the side of an imaging member bearing the imaging layers. The terms "bottom", "lower side", and "back" mean the side or towards the side of the imaging member opposite from the side bearing the imaging layers or developed image. The term "tie layer" as used herein refers to a layer of material that is used to adhere biaxially oriented sheets to a base such as paper, polyester, fabric, or other suitable material for the viewing of images.

The photographic element that provides improved resistance to high pressure forces on the backside comprises at least one silver halide and dye forming coupler containing imaging layer and a cushioning layer below at least one side imaging layer having a deformable tie layer material, wherein said deformable material having a yield stress in compression less than 10% of any of the other layers in the element. The deformable material suitably has a plastic deformation stress of between 6 and 10 MPa. The other image base materials have a plastic deformation of between about 60 and 100 MPa. The most preferred deformable material has plastic deformation stress of 8 MPa and comprises a medium density polyethylene (density 0.926) at least 20  $\mu\text{m}$  thick. Medium density polyethylene is hereby defined as having a density range, before extrusion, of 0.926 to 0.940. Other polyolefin layers having a plastic deformation stress below 10 MPa are also suitable. These may include polyethylene, polypropylene, ethylene-vinyl acetate, polybutylene, polymethylpentene, and polydicyclopentadiene. The cushioned layer, as incorporated in this invention, allows the backside compressive forces to be applied to a deformable layer that, once deformed, reduces the pressure on the silver grains and significantly reducing the deformation of the emulsion and any deformable tie layers on the emulsion side, thereby preventing surface imperfections. It is important that the cushioning layer undergoes an inelastic deformation and does not rebound or recover from the applied load.

The preferred location of deformable layer is below the oriented voided polyolefin sheet and under the photographic emulsion and as far as possible from the emulsion. This location is preferred because the deformable layer is most effective when it is located near the applied pressure. In this

65

situation the force being applied to the emulsion can be more effectively dissipated. It is also possible to either add a second cushioning layer to the bottom side of a photographic element or to use the backside location as the sole cushion layer. Additional improvements may be realized with additional layers on the same side or in combination on the top and bottom sides of the base substrate.

The photographic element containing a biaxially oriented voided polyolefin sheet is normally adhered to a paper base by a lamination process. The preferred embodiment of this invention uses a melt extrudable polyolefin polymer to adhere the sheet to the paper base. Melt extrudable polyolefin polymers are used because of their relative low cost, stability, chemical inertness, and general ease of handling. Depending on the end use of the photographic element, it may be desirable to use a polyester base substrate in place of paper. In this case, a laminated cushion layer is critical because the polyester base has little or no compressibility in the thickness direction, and there is a greater need to have a force reducing layer to minimize pressure induced imperfections.

The sensitivity of a photographic emulsion layer containing silver halide may be impacted by a variety of parameters such as silver grain size, the ratio of silver grains to binder, as well as the addition of chemical addenda.

A deformable layer may also be formed by chemical or physical blowing agents. Typical materials comprise one or more from the list of azodicarbonamide, zeolite or molecular sieves, gases such as nitrogen, carbon dioxide or liquids that turn to gas at atmospheric pressure.

Any suitable biaxially oriented polyolefin sheet may be used for the sheet on the top side of the laminated base used in the invention. Microvoided composite biaxially oriented sheets are preferred and are conveniently manufactured by coextrusion of the core and surface layers, followed by biaxial orientation, whereby voids are formed around void-initiating material contained in the core layer. Such composite sheets may be formed as in U.S. Pat. Nos. 4,377,616; 4,758,462; and 4,632,869.

The core of the preferred composite sheet should be from 15 to 95% of the total thickness of the sheet, preferably from 30 to 85% of the total thickness. The nonvoided skin(s) should thus be from 5 to 85% of the sheet, preferably from 15 to 70% of the thickness.

The density (specific gravity) of the composite sheet, expressed in terms of "percent of solid density" is calculated as follows:

$$\frac{\text{Composite Sheet Density}}{\text{Polymer Density}} \times 100 = \% \text{ of Solid Density}$$

Percent solid density should be between 45% and 100%, preferably between 67% and 100%. As the percent solid density becomes less than 67%, the composite sheet becomes less manufacturable due to a drop in tensile strength and it becomes more susceptible to physical damage.

The total thickness of the composite sheet can range from 12 to 100  $\mu\text{m}$ , preferably from 20 to 70  $\mu\text{m}$ . Below 20  $\mu\text{m}$ , the microvoided sheets may not be thick enough to minimize any inherent non-planarity in the support and would be more difficult to manufacture. At thickness higher than 70  $\mu\text{m}$ , little improvement in either surface smoothness or mechanical properties are seen, and so there is little justification for the further increase in cost for extra materials.

The biaxially oriented sheets of the invention preferably have a water vapor permeability that is less than  $0.85 \times 10^{-5}$  g/mm<sup>2</sup>/day. This allows faster emulsion hardening, as the laminated support of this invention greatly slows the rate of water vapor transmission from the emulsion layers during coating of the emulsions on the support. The transmission rate is measured by ASTM F1249.

"Void" is used herein to mean devoid of added solid and liquid matter, although it is likely the "voids" contain gas. The void-initiating particles which remain in the finished packaging sheet core should be from 0.1 to 10  $\mu\text{m}$  in diameter, preferably round in shape, to produce voids of the desired shape and size. The size of the void is also dependent on the degree of orientation in the machine and transverse directions. Ideally, the void would assume a shape which is defined by two opposed and edge contacting concave disks. In other words, the voids tend to have a lens-like or biconvex shape. The voids are oriented so that the two major dimensions are aligned with the machine and transverse directions of the sheet. The Z-direction axis is a minor dimension and is roughly the size of the cross diameter of the voiding particle. The voids generally tend to be closed cells, and thus there is virtually no path open from one side of the voided-core to the other side through which gas or liquid can traverse.

25 The void-initiating material may be selected from a variety of materials, and should be present in an amount of about 5 to 50% by weight based on the weight of the core matrix polymer. Preferably, the void-initiating material comprises a polymeric material. When a polymeric material is used, it may be a polymer that can be melt-mixed with the polymer from which the core matrix is made and be able to form dispersed spherical particles as the suspension is cooled down. Examples of this would include nylon dispersed in polypropylene, polybutylene terephthalate in 30 polypropylene, or polypropylene dispersed in polyethylene terephthalate. If the polymer is preshaped and blended into the matrix polymer, the important characteristic is the size and shape of the particles. Spheres are preferred and they can be hollow or solid. These spheres may be made from 35 cross-linked polymers which are members selected from the group consisting of an alkenyl aromatic compound having the general formula Ar—C(R)=CH<sub>2</sub>, wherein Ar represents an aromatic hydrocarbon radical, or an aromatic halohydrocarbon radical of the benzene series and R is hydrogen or the 40 methyl radical; acrylate-type monomers include monomers of the formula CH<sub>2</sub>=C(R')—C(O)(OR) wherein R is selected from the group consisting of hydrogen and an alkyl radical containing from about 1 to 12 carbon atoms and R' is selected from the group consisting of hydrogen and 45 methyl; copolymers of vinyl chloride and vinylidene chloride, acrylonitrile and vinyl chloride, vinyl bromide, vinyl esters having formula CH<sub>2</sub>=CH(O)COR, wherein R is an alkyl radical containing from 2 to 18 carbon atoms; acrylic acid, methacrylic acid, itaconic acid, citraconic acid, 50 maleic acid, fumaric acid, oleic acid, vinylbenzoic acid; the synthetic polyester resins which are prepared by reacting terephthalic acid and dialkyl terephthalates or ester-forming derivatives thereof, with a glycol of the series HO(CH<sub>2</sub>)<sub>n</sub>OH wherein n is a whole number within the range of 2-10 and 55 having reactive olefinic linkages within the polymer molecule, the above described polyesters which include copolymerized therein up to 20 percent by weight of a second acid or ester thereof having reactive olefinic unsaturation and mixtures thereof, and a cross-linking agent 60 selected from the group consisting of divinylbenzene, diethylene glycol dimethacrylate, diallyl fumarate, diallyl phthalate and mixtures thereof.

Examples of typical monomers for making the crosslinked polymer include styrene, butyl acrylate, acrylamide, acrylonitrile, methyl methacrylate, ethylene glycol dimethacrylate, vinyl pyridine, vinyl acetate, methyl acrylate, vinylbenzyl chloride, vinylidene chloride, acrylic acid, divinylbenzene, acrylamidomethyl-propane sulfonic acid, vinyl toluene, etc. Preferably, the cross-linked polymer is polystyrene or poly(methyl methacrylate). Most preferably, it is polystyrene and the cross-linking agent is divinylbenzene.

Processes well known in the art yield non-uniformly sized particles, characterized by broad particle size distributions. The resulting beads can be classified by screening the beads spanning the range of the original distribution of sizes. Other processes such as suspension polymerization, limited coalescence, directly yield very uniformly sized particles.

The void-initiating materials may be coated with agents to facilitate voiding. Suitable agents or lubricants include colloidal silica, colloidal alumina, and metal oxides such as tin oxide and aluminum oxide. The preferred agents are colloidal silica and alumina, most preferably, silica. The cross-linked polymer having a coating of an agent may be prepared by procedures well known in the art. For example, conventional suspension polymerization processes wherein the agent is added to the suspension is preferred. As the agent, colloidal silica is preferred.

The void-initiating particles can also be inorganic spheres, including solid or hollow glass spheres, metal or ceramic beads or inorganic particles such as clay, talc, barium sulfate, calcium carbonate. The important thing is that the material does not chemically react with the core matrix polymer to cause one or more of the following problems: (a) alteration of the crystallization kinetics of the matrix polymer, making it difficult to orient, (b) destruction of the core matrix polymer, (c) destruction of the void-initiating particles, (d) adhesion of the void-initiating particles to the matrix polymer, or (e) generation of undesirable reaction products, such as toxic or high color moieties. The void-initiating material should not be photographically active or degrade the performance of the photographic element in which the biaxially oriented polyolefin sheet is utilized.

For the biaxially oriented sheet on the top side toward the emulsion, suitable classes of thermoplastic polymers for the biaxially oriented sheet and the core matrix-polymer of the preferred composite sheet comprise polyolefins.

Suitable polyolefins include polypropylene, polyethylene, polymethylpentene, polystyrene, polybutylene, and mixtures thereof. Polyolefin copolymers, including copolymers of propylene and ethylene such as hexene, butene, and octene are also useful. Polypropylene is preferred, as it is low in cost and has desirable strength properties.

The nonvoided skin layers of the composite sheet can be made of the same polymeric materials as listed above for the core matrix. The composite sheet can be made with skin(s) of the same polymeric material as the core matrix, or it can be made with skin(s) of different polymeric composition than the core matrix. For compatibility, an auxiliary layer can be used to promote adhesion of the skin layer to the core.

Addenda may be added to the core matrix and/or to the skins to improve the whiteness of these sheets. This would include any process which is known in the art including adding a white pigment, such as titanium dioxide, barium sulfate, clay, or calcium carbonate. This would also include adding fluorescing agents which absorb energy in the UV region and emit light largely in the blue region, or other

additives which would improve the physical properties of the sheet or the manufacturability of the sheet. For photographic use, a white base with a slight bluish tint is preferred.

5 The coextrusion, quenching, orienting, and heat setting of these composite sheets may be effected by any process which is known in the art for producing oriented sheet, such as by a flat sheet process or a bubble or tubular process. The flat sheet process involves extruding the blend through a slit 10 die and rapidly quenching the extruded web upon a chilled casting drum so that the core matrix polymer component of the sheet and the skin components(s) are quenched below their glass solidification temperature. The quenched sheet is then biaxially oriented by stretching in mutually perpendicular directions at a temperature above the glass transition temperature, below the melting temperature of the matrix polymers. The sheet may be stretched in one direction and then in a second direction or may be simultaneously stretched in both directions. After the sheet has been 15 stretched, it is heat set by heating to a temperature sufficient to crystallize or anneal the polymers while restraining to some degree the sheet against retraction in both directions of stretching.

20 The composite sheet, while described as having preferably at least three layers of a microvoided core and a skin layer on each side, may also be provided with additional layers that may serve to change the properties of the biaxially oriented sheet. A different effect may be achieved by additional layers. Such layers might contain tints, antistatic materials, or different void-making materials to produce sheets of unique properties. Biaxially oriented sheets could be formed with surface layers that would provide an improved adhesion, or look to the support and photographic element. The biaxially oriented extrusion could be carried 25 out with as many as 10 or more layers if desired to achieve some particular desired property.

These composite sheets may be coated or treated after the coextrusion and orienting process or between casting and full orientation with any number of coatings which may be 30 used to improve the properties of the sheets including printability, to provide a vapor barrier, to make them heat sealable, or to improve the adhesion to the support or to the photo sensitive layers. Examples of this would be acrylic coatings for printability, coating polyvinylidene chloride for 35 heat seal properties. Further examples include flame, plasma or corona discharge treatment to improve printability or adhesion.

40 By having at least one nonvoided skin on the microvoided core, the tensile strength of the sheet is increased and makes it more manufacturable. It allows the sheets to be made at wider widths and higher draw ratios than when sheets are made with all layers voided. Coextruding the layers further 45 simplifies the manufacturing process.

50 The structure of a typical biaxially oriented, sheet of the invention is as follows:



55 The sheet on the side of the base paper opposite to the emulsion layers may be any suitable sheet. The sheet may or 60 may not be microvoided. It may have the same composition as the sheet on the top side of the paper backing material.

Biaxially oriented sheets are conveniently manufactured by coextrusion of the sheet, which may contain several layers, followed by biaxial orientation. Such biaxially oriented sheets are disclosed in, for example, U.S. Pat. No. 4,764,425.

The preferred biaxially oriented sheet is a biaxially oriented polyolefin sheet, most preferably a sheet of polyethylene or polypropylene. The thickness of the biaxially oriented sheet should be from 10 to 150  $\mu\text{m}$ . Below 15  $\mu\text{m}$ , the sheets may not be thick enough to minimize any inherent non-planarity in the support and would be more difficult to manufacture. At thicknesses higher than 70  $\mu\text{m}$ , little improvement in either surface smoothness or mechanical properties are seen, and so there is little justification for the further increase in cost for extra materials.

Suitable classes of thermoplastic polymers for the biaxially oriented sheet include polyolefins, polyesters, polyamides, polycarbonates, cellulosic esters, polystyrene, polyvinyl resins, polysulfonamides, polyethers, polyimides, polyvinylidene fluoride, polyurethanes, polyphenylenesulfides, polytetrafluoroethylene, polyacetals, polysulfonates, polyester ionomers, and polyolefin ionomers. Copolymers and/or mixtures of these polymers can be used.

Suitable polyolefins include polypropylene, polyethylene, polymethylpentene, and mixtures thereof. Polyolefin copolymers, including copolymers of propylene and ethylene such as hexene, butene and octene are also useful. Polypropylenes are preferred because they are low in cost and have good strength and surface properties.

Suitable polyesters include those produced from aromatic, aliphatic or cycloaliphatic dicarboxylic acids of 4-20 carbon atoms and aliphatic or alicyclic glycols having from 2-24 carbon atoms. Examples of suitable dicarboxylic acids include terephthalic, isophthalic, phthalic, naphthalene dicarboxylic acid, succinic, glutaric, adipic, azelaic, sebacic, fumaric, maleic, itaconic, 1,4-cyclohexanedicarboxylic, sodiosulfoisophthalic and mixtures thereof. Examples of suitable glycols include ethylene glycol, propylene glycol, butanediol, pentanediol, hexanediol, 1,4-cyclohexanediethanol, diethylene glycol, other polyethylene glycols and mixtures thereof. Such polyesters are well known in the art and may be produced by well-known techniques, e.g., those described in U.S. Pat. Nos. 2,465,319 and U.S. Pat. No. 2,901,466. Preferred continuous matrix polyesters are those having repeat units from terephthalic acid or naphthalene dicarboxylic acid and at least one glycol selected from ethylene glycol, 1,4-butanediol and 1,4-cyclohexanediethanol. Poly(ethylene terephthalate), which may be modified by small amounts of other monomers, is especially preferred. Other suitable polyesters include liquid crystal copolymers formed by the inclusion of suitable amount of a co-acid component such as stilbene dicarboxylic acid. Examples of such liquid crystal copolymers are those disclosed in U.S. Pat. Nos. 4,420,607; 4,459,402; and 4,468,510.

Useful polyamides include nylon 6, nylon 66, and mixtures thereof. Copolymers of polyamides are also suitable continuous phase polymers. An example of a useful polycarbonate is bisphenol-A polycarbonate. Cellulosic esters suitable for use as the continuous phase polymer of the composite sheets include cellulose nitrate, cellulose triacetate, cellulose diacetate, cellulose acetate propionate, cellulose acetate butyrate, and mixtures or copolymers thereof. Useful polyvinyl resins include polyvinyl chloride, poly(vinyl acetal), and mixtures thereof. Copolymers of vinyl resins can also be utilized.

The biaxially oriented sheet on the backside of the laminated base can be made with layers of the same polymeric material, or it can be made with layers of different polymeric composition. For compatibility, an auxiliary layer can be used to promote adhesion of multiple layers.

Addenda may be added to the biaxially oriented backside sheet to improve the whiteness of these sheets. This would include any process which is known in the art including adding a white pigment, such as titanium dioxide, barium sulfate, clay, or calcium carbonate. This would also include adding fluorescing agents which absorb energy in the UV region and emit light largely in the blue region, or other additives which would improve the physical properties of the sheet or the manufacturability of the sheet.

The coextrusion, quenching, orienting, and heat setting of these biaxially oriented sheets may be effected by any process which is known in the art for producing oriented sheet, such as by a flat sheet process or a bubble or tubular process. The flat sheet process involves extruding or coextruding the blend through a slit die and rapidly quenching the extruded or coextruded web upon a chilled casting drum so that the polymer component(s) of the sheet are quenched below their solidification temperature. The quenched sheet is then biaxially oriented by stretching in mutually perpendicular directions at a temperature above the glass transition temperature of the polymer(s). The sheet may be stretched in one direction and then in a second direction or may be simultaneously stretched in both directions. After the sheet has been stretched, it is heat set by heating to a temperature sufficient to crystallize the polymers while restraining to some degree the sheet against retraction in both directions of stretching.

The biaxially oriented sheet on the backside of the laminated base, while described as having preferably at least one layer, may also be provided with additional layers that may serve to change the properties of the biaxially oriented sheet. A different effect may be achieved by additional layers. Such layers might contain tints, antistatic materials, or slip agents to produce sheets of unique properties. Biaxially oriented sheets could be formed with surface layers that would provide an improved adhesion, or look to the support and photographic element. The biaxially oriented extrusion could be carried out with as many as 10 layers if desired to achieve some particular desired property.

These biaxially oriented sheets may be coated or treated after the coextrusion and orienting process or between casting and full orientation with any number of coatings which may be used to improve the properties of the sheets including printability, to provide a vapor barrier, to make them heat sealable, or to improve the adhesion to the support or to the photo sensitive layers. Examples of this would be acrylic coatings for printability, coating polyvinylidene chloride for heat seal properties. Further examples include flame, plasma or corona discharge treatment to improve printability or adhesion.

The structure of a typical biaxially oriented sheet that may be laminated to the opposite side of the imaging elements is as follows:



The support to which the microvoided composite sheets and biaxially oriented sheets are laminated for the laminated

support of the photosensitive silver halide layer may be a polymeric, a synthetic paper, cloth, woven polymer fibers, or a cellulose fiber paper support, or laminates thereof. The base also may be a microvoided polyethylene terephthalate such as disclosed in U.S. Pat. Nos. 4,912,333; 4,994,312; and 5,055,371.

The preferred support is a photographic grade cellulose fiber paper. When using a cellulose fiber paper support, it is preferable to extrusion laminate the microvoided composite sheets to the base paper using a polyolefin resin. Extrusion laminating is carried out by bringing together the biaxially oriented sheets of the invention and the base paper with application of an adhesive between them followed by their being pressed in a nip such as between two rollers. The adhesive may be applied to either the biaxially oriented sheets or the base paper prior to their being brought into the nip. In a preferred form, the adhesive is applied into the nip simultaneously with the biaxially oriented sheets and the base paper. The adhesive may be any suitable material that does not have a harmful effect upon the photographic element. A preferred material is polyethylene that is melted at the time it is placed into the nip between the paper and the biaxially oriented sheet.

During the lamination process, it is desirable to maintain control of the tension of the biaxially oriented sheets in order to minimize curl in the resulting laminated support. For high humidity applications (>50% RH) and low humidity applications (<20% RH), it is desirable to laminate both a front side and back side film to keep curl to a minimum.

The surface roughness of this invention can also be accomplished by laminating a biaxially oriented sheet to a paper base that has the desired roughness. The roughness of the paper base can be accomplished by any method known in the art such as a heated impression nip or a press felt combined with a roller nip in which the rough surface is part of the press nip. The preferred roughness of the base paper is from 35  $\mu\text{m}$  to 150  $\mu\text{m}$ . This preferred range is larger than roughness range for the imaging support because of the loss of roughness that occurs in melt extrusion lamination.

In one preferred embodiment, in order to produce photographic elements with a desirable photographic look and feel, it is preferable to use relatively thick paper supports (e.g., at least 120  $\mu\text{m}$  thick, preferably from 120 to 250  $\mu\text{m}$  thick) and relatively thin microvoided composite sheets (e.g., less than 50  $\mu\text{m}$  thick, preferably from 20 to 50  $\mu\text{m}$  thick, more preferably from 30 to 50  $\mu\text{m}$  thick).

As used herein, the phrase "photographic element" is a material that utilizes photosensitive silver halide in the formation of images. In the case of thermal dye transfer or ink jet, the image layer that is coated on the imaging element may be any material that is known in the art such as gelatin, pigmented latex, polyvinyl alcohol, polycarbonate, polyvinyl pyrrolidone, starch, and methacrylate. The photographic elements can be single color elements or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

The photographic emulsions useful for this invention are generally prepared by precipitating silver halide crystals in a colloidal matrix by methods conventional in the art. The

colloid is typically a hydrophilic film forming agent such as gelatin, alginic acid, or derivatives thereof.

The crystals formed in the precipitation step are washed and then chemically and spectrally sensitized by adding spectral sensitizing dyes and chemical sensitizers, and by providing a heating step during which the emulsion temperature is raised, typically from 40° C. to 70° C., and maintained for a period of time. The precipitation and spectral and chemical sensitization methods utilized in preparing the emulsions employed in the invention can be those methods known in the art.

Chemical sensitization of the emulsion typically employs sensitizers such as: sulfur-containing compounds, e.g., allyl isothiocyanate, sodium thiosulfate and allyl thiourea; reducing agents, e.g., polyamines and stannous salts; noble metal compounds, e.g., gold, platinum; and polymeric agents, e.g., polyalkylene oxides. As described, heat treatment is employed to complete chemical sensitization. Spectral sensitization is effected with a combination of dyes, which are designed for the wavelength range of interest within the visible or infrared spectrum. It is known to add such dyes both before and after heat treatment.

After spectral sensitization, the emulsion is coated on a support. Various coating techniques include dip coating, air knife coating, curtain coating and extrusion coating.

The silver halide emulsions utilized in this invention may be comprised of any halide distribution. Thus, they may be comprised of silver chloride, silver chloroiodide, silver bromide, silver bromochloride, silver chlorobromide, silver iodochloride, silver iodobromide, silver bromoiodochloride, silver chloroiodobromide, silver iodobromochloride, and silver iodochlorobromide emulsions. It is preferred, however, that the emulsions be predominantly silver chloride emulsions. By predominantly silver chloride, it is meant that the grains of the emulsion are greater than about 50 mole percent silver chloride. Preferably, they are greater than about 90 mole percent silver chloride; and optimally greater than about 95 mole percent silver chloride.

The silver halide emulsions can contain grains of any size and morphology. Thus, the grains may take the form of cubes, octahedrons, cubo-octahedrons, or any of the other naturally occurring morphologies of cubic lattice type silver halide grains. Further, the grains may be irregular such as spherical grains or tabular grains. Grains having a tabular or cubic morphology are preferred.

The photographic elements of the invention may utilize emulsions as described in *The Theory of the Photographic Process*, Fourth Edition, T. H. James, Macmillan Publishing Company, Inc., 1977, pages 151–152. Reduction sensitization has been known to improve the photographic sensitivity of silver halide emulsions. While reduction sensitized silver halide emulsions generally exhibit good photographic speed, they often suffer from undesirable fog and poor storage stability.

Reduction sensitization can be performed intentionally by adding reduction sensitizers, chemicals which reduce silver ions to form metallic silver atoms, or by providing a reducing environment such as high pH (excess hydroxide ion) and/or low pAg (excess silver ion). During precipitation of a silver halide emulsion, unintentional reduction sensitization can occur when, for example, silver nitrate or alkali solutions are added rapidly or with poor mixing to form emulsion grains. Also, precipitation of silver halide emulsions in the presence of ripeners (grain growth modifiers) such as thioethers, selenoethers, thioureas, or ammonia tends to facilitate reduction sensitization.

Examples of reduction sensitizers and environments which may be used during precipitation or spectral/chemical sensitization to reduction sensitize an emulsion include ascorbic acid derivatives; tin compounds; polyamine compounds; and thiourea dioxide-based compounds described in U.S. Pat. Nos. 2,487,850; 2,512,925; and British Patent 789,823. Specific examples of reduction sensitizers or conditions, such as dimethylamineborane, stannous chloride, hydrazine, high pH (pH 8–11) and low pAg (pAg 1–7) ripening are discussed by S. Collier in *Photographic Science and Engineering*, 23, 113 (1979). Examples of processes for preparing intentionally reduction sensitized silver halide emulsions are described in EP 0 348 934 A1 (Yamashita), EP 0 369 491 (Yamashita), EP 0 371 388 (Ohashi), EP 0 396 424 A1 (Takada), EP 0 404 142 A1 (Yamada), and EP 0 435 355 A1 (Makino).

The photographic elements of this invention may use emulsions doped with Group VIII metals such as iridium, rhodium, osmium, and iron as described in *Research Disclosure*, September 1996, Item 38957, Section I, published by Kenneth Mason Publications, Ltd., Dudley Annex, 12a North Street, Emsworth, Hampshire PO10 7DQ, ENGLAND. Additionally, a general summary of the use of iridium in the sensitization of silver halide emulsions is contained in Carroll, "Iridium Sensitization: A Literature Review," *Photographic Science and Engineering*, Vol. 24, No. 6, 1980. A method of manufacturing a silver halide emulsion by chemically sensitizing the emulsion in the presence of an iridium salt and a photographic spectral sensitizing dye is described in U.S. Pat. No. 4,693,965. In some cases, when such dopants are incorporated, emulsions show an increased fresh fog and a lower contrast sensitometric curve when processed in the color reversal E-6 process as described in *The British Journal of Photography Annual*, 1982, pages 201–203.

A typical multicolor photographic element of the invention comprises the invention laminated support bearing a cyan dye image-forming unit comprising at least one red-sensitive silver halide emulsion layer having associated therewith at least one cyan dye-forming coupler; a magenta image-forming unit comprising at least one green-sensitive silver halide emulsion layer having associated therewith at least one magenta dye-forming coupler; and a yellow dye image-forming unit comprising at least one blue-sensitive silver halide emulsion layer having associated therewith at least one yellow dye-forming coupler. The element may contain additional layers, such as filter layers, interlayers, overcoat layers, subbing layers, and the like. The support of the invention may also be utilized for black and white photographic print elements.

The photographic elements may also contain a transparent magnetic recording layer such as a layer containing magnetic particles on the underside of a transparent support, as in U.S. Pat. Nos. 4,279,945 and 4,302,523. Typically, the element will have a total thickness (excluding the support) of from about 5 to about 30  $\mu\text{m}$ .

In the following Table, reference will be made to (1) *Research Disclosure*, December 1978, Item 17643, (2) *Research Disclosure*, December 1989, Item 308119, and (3) *Research Disclosure*, September 1996, Item 38957, all published by Kenneth Mason Publications, Ltd., Dudley Annex, 12 a North Street, Emsworth, Hampshire PO10 7DQ, ENGLAND. The Table and the references cited in the Table are to be read as describing particular components suitable for use in the elements of the invention. The Table and its cited references also ways of preparing, exposing, processing and manipulating the images contained therein.

| Reference | Section                          | Subject Matter                                                                 |
|-----------|----------------------------------|--------------------------------------------------------------------------------|
| 5         | 1 I, II                          | Grain composition, morphology and preparation.                                 |
|           | 2 I, II, IX, X, XI, XII, XIV, XV | Emulsion preparation including hardeners, coating aids, addenda, etc.          |
|           | 3 I, II, III, IX A & B           | Chemical sensitization and spectral sensitization/desensitization              |
| 10        | 1 III, IV                        | UV dyes, optical brighteners, luminescent dyes                                 |
|           | 2 III, IV                        | Antifoggants and stabilizers                                                   |
|           | 3 IV, V                          |                                                                                |
|           | 1 V                              | Absorbing and scattering materials; Antistatic layers; matting agents          |
|           | 2 V                              | Image-couplers and image-modifying couplers; Dye stabilizers and hue modifiers |
|           | 3 VI                             | Supports                                                                       |
| 15        | 1 VI                             |                                                                                |
|           | 2 VI                             | Specific layer arrangements                                                    |
|           | 3 VII                            | Negative working emulsions; Direct positive emulsions                          |
| 20        | 1 VII                            | Exposure                                                                       |
|           | 2 VIII, XIII, XVI                | Chemical processing; Developing agents                                         |
|           | 3 VIII, IX C & D                 |                                                                                |
| 25        | 1 VII                            | Scanning and digital processing procedures                                     |
|           | 2 VII                            |                                                                                |
|           | 3 X                              |                                                                                |
|           | 1 XVII                           |                                                                                |
|           | 2 XVII                           |                                                                                |
|           | 3 XV                             |                                                                                |
| 30        | 1 XI                             |                                                                                |
|           | 3 XII, XIII                      |                                                                                |
| 35        | 2 XVIII                          |                                                                                |
|           | 3 XVI                            |                                                                                |
|           | 1 XIX, XX                        |                                                                                |
|           | 2 XIX, XX, XXII                  |                                                                                |
|           | 3 XVIII, XIX, XX                 |                                                                                |
| 40        | 3 XIV                            |                                                                                |

The photographic elements can be exposed with various forms of energy which encompass the ultraviolet, visible, and infrared regions of the electromagnetic spectrum as well as with electron beam, beta radiation, gamma radiation, x-ray, alpha particle, neutron radiation, and other forms of corpuscular and wave-like radiant energy in either noncoherent (random phase) forms or coherent (in phase) forms, as produced by lasers. When the photographic elements are intended to be exposed by x-rays, they can include features found in conventional radiographic elements.

The photographic elements are preferably exposed to actinic radiation, typically in the visible region of the spectrum, to form a latent image, and then processed to form a visible image, preferably by other than heat treatment. Processing is preferably carried out in the known RA-4™ (Eastman Kodak Company) Process or other processing systems suitable for developing high chloride emulsions.

The laminated substrate of the invention may have copy restriction features incorporated such as disclosed in U.S. Pat. Nos. 5,752,152 and 5,919,730. These applications disclose rendering a document copy restrictive by embedding into the document a pattern of invisible microdots. These microdots are, however, detectable by the electro-optical scanning device of a digital document copier. The pattern of microdots may be incorporated throughout the document. Such documents may also have colored edges or an invisible microdot pattern on the back side to enable users or machines to read and identify the media. The media may take the form of sheets that are capable of bearing an image. Typical of such materials are photographic paper and film materials composed of polyethylene resin coated paper, polyester, (poly)ethylene naphthalate, and cellulose triacetate based materials.

The microdots can take any regular or irregular shape with a size smaller than the maximum size at which indi-

vidual microdots are perceived sufficiently to decrease the usefulness of the image, and the minimum level is defined by the detection level of the scanning device. The microdots may be distributed in a regular or irregular array with center-to-center spacing controlled to avoid increases in document density. The microdots can be of any hue, brightness, and saturation that does not lead to sufficient detection by casual observation, but preferably of a hue least resolvable by the human eye, yet suitable to conform to the sensitivities of the document scanning device for optimal detection.

In one embodiment the information-bearing document is comprised of a support, an image-forming layer coated on the support and pattern of microdots positioned between the support and the image-forming layer to provide a copy restrictive medium. Incorporation of the microdot pattern into the document medium can be achieved by various printing technologies either before or after production of the original document. The microdots can be composed of any colored substance, although depending on the nature of the document, the colorants may be translucent, transparent, or opaque. It is preferred to locate the microdot pattern on the support layer prior to application of the protective layer, unless the protective layer contains light scattering pigments. Then the microdots should be located above such layers and preferably coated with a protective layer. The microdots can be composed of colorants chosen from image dyes and filter dyes known in the photographic art and dispersed in a binder or carrier used for printing inks or light-sensitive media.

In a preferred embodiment the creation of the microdot pattern as a latent image is possible through appropriate temporal, spatial, and spectral exposure of the photosensitive materials to visible or non-visible wavelengths of electromagnetic radiation. The latent image microdot pattern can be rendered detectable by employing standard photographic chemical processing. The microdots are particularly useful for both color and black-and-white image-forming photographic media. Such photographic media will contain at least one silver halide radiation sensitive layer, although typically such photographic media contain at least three silver halide radiation sensitive layers. It is also possible that such media contain more than one layer sensitive to the same region of radiation. The arrangement of the layers may take any of the forms known to one skilled in the art, as discussed in *Research Disclosure* 37038 of February 1995.

The following examples illustrate the practice of this invention. They are not intended to be exhaustive of all possible variations of the invention. Parts and percentages are by weight unless otherwise indicated.

#### Commercial Grade Paper of Examples

A photographic paper support was produced by refining a pulp furnish of 50% bleached hardwood kraft, 25% bleached hardwood sulfite, and 25% bleached softwood sulfite through a double disk refiner, then a Jordan conical refiner to a Canadian Standard Freeness of 200 cc. To the resulting pulp furnish was added 0.2% alkyl ketene dimer, 1.0% cationic cornstarch, 0.5% polyamide-epichlorohydrin, 0.26 anionic polyacrylamide, and 5.0% TiO<sub>2</sub> on a dry weight basis. An about 46.5 lbs. per 1000 sq. ft. (ksf) bone dry weight base paper was made on a fourdrinier paper machine, wet pressed to a solid of 42%, and dried to a moisture of 10% using steam-heated dryers achieving a Sheffield Porosity of 160 Sheffield Units and an apparent density 0.70 g/cc. The paper base was then surface sized using a vertical size

press with a 10% hydroxyethylated cornstarch solution to achieve a loading of 3.3 wt. % starch. The surface sized support was calendered to an apparent density of 1.04 gm/cc.

The following examples illustrate the practice of this invention. They are not intended to be exhaustive of all possible variations of the invention. Parts and percentages are by weight unless otherwise indicated.

#### EXAMPLE

The following laminated photographic bases were prepared by extrusion laminating a biaxially oriented sheets with voids to the emulsion side of the photographic grade cellulose paper base and one biaxially oriented sheets to the back side of the photographic grade cellulose paper base:

A composite top sheet consisting of 5 layers identified as L1, L2, L3, L4, and L5. L1 is the thin colored layer on the outside of the package to which the photosensitive silver halide layer was attached. L6 was the extrusion coated adhesive layer used to laminate the top sheet to the paper support. L8 was the extrusion coated adhesive layer used to laminate the bottom sheet to the paper support.

The top sheet was coextruded and biaxially oriented by MOBIL Chemical Co. similar to the process used to make commercially available OPPalyte 350TW. Table 1 shows the layer structure for this example.

TABLE 1



Table 2 lists the further characteristics of the samples.

TABLE 2

| Layer | Material                                   | Thickness, $\mu\text{m}$ |
|-------|--------------------------------------------|--------------------------|
| L1    | LD Polyethylene                            | 1.5                      |
| L2    | Polypropylene + 18% TiO <sub>2</sub> by wt | 4.32                     |
| L3    | Voided Polypropylene                       | 24.9                     |
| L4    | Polypropylene                              | 4.32                     |
| L5    | Polypropylene                              | 0.762                    |
| L6    | LD Polyethylene tie layer                  | variable                 |
| L7    | Commercial paper base                      | 142                      |
| L8    | Deforming tie layer                        | variable                 |

The L3 layer is microvoided and further described in Table 3 where the refractive index and geometrical thickness is shown for measurements made along a single slice through the L3 layer; they do not imply continuous layers, a slice along another location would yield different but approxi-

## 15

mately the same thickness. The area with a refractive index of 1 are voids that are filled with air, and the remaining layers polypropylene.

TABLE 3

| Sublayer of L3 | Refractive Index | Thickness, $\mu\text{m}$ |
|----------------|------------------|--------------------------|
| 1              | 1.49             | 2.54                     |
| 2              | 1                | 1.527                    |
| 3              | 1.49             | 2.79                     |
| 4              | 1                | 1.016                    |
| 5              | 1.49             | 1.778                    |
| 6              | 1                | 1.016                    |
| 7              | 1.49             | 2.286                    |
| 8              | 1                | 1.016                    |
| 9              | 1.49             | 2.032                    |
| 10             | 1                | 0.762                    |
| 11             | 1.49             | 2.032                    |
| 12             | 1                | 1.016                    |
| 13             | 1.49             | 1.778                    |
| 14             | 1                | 1.016                    |
| 15             | 1.49             | 2.286                    |

The bottom sheet was BICOR 70 MLT from Mobil Chemical Co., a one-side matte finish, one-side treated polypropylene sheet (18  $\mu\text{m}$  thick) ( $d=0.9 \text{ g/cc}$ ) consisting of a cold oriented polypropylene core.

The samples for the example were obtained by changing L6 and L8 tie layer caliper as shown in Table 4. Samples 1–6 are controls, and Sample 7 is an invention sample.

TABLE 4

| Sample | L6 caliper, $\mu\text{m}$ | L8 caliper, $\mu\text{m}$ | Surface deformation observed |
|--------|---------------------------|---------------------------|------------------------------|
| 1      | 11.4                      | 11.4                      | yes                          |
| 2      | 6.9                       | 11.4                      | yes                          |
| 3      | 18.3                      | 11.4                      | yes                          |
| 4      | 11.4                      | 15.1                      | yes                          |
| 5      | 11.4                      | 19.0                      | yes                          |
| 6      | 6.9                       | 18.3                      | yes                          |
| 7      | 11.4                      | 21.5                      | No                           |

The testing for sensitivity to pressures simulating a dot matrix printer or other high pressure printers was accomplished by the use of a knurled wheel pressing on the backside of the samples. The wheel was a metal knurling device number KPS-240-90 40 tpi purchased from the Formroll Company. The wheel had triangular sharp 90 degree angle teeth spaced 0.635 mm apart and a tooth depth of 0.635 mm. The teeth were 10 mm wide. The wheel was applied to the sample backside with a force of 473 newton through an air cylinder. The samples were mechanically transported under the knurling wheel and against a hard surface at a speed of 0.5 m/sec. The samples were visually

## 16

inspected and the surface was also measured by topographical tracing equipment to determine if any undesirable surface deformation was present.

An L8 layer caliper of greater than 20  $\mu\text{m}$  was required to prevent surface deformation.

The invention has been described in detail with particular reference to certain preferred embodiments thereof, but it will be understood that variations and modifications can be effected within the spirit and scope of the invention.

## What is claimed is:

1. A photographic element comprising at least one layer of photosensitive silver halide, a base material wherein said base material comprises at least one bottom sheet of biaxially oriented polymer sheet and deformable tie layer material, wherein said deformable tie layer material yield stress of between 6 and 10 MPa in compression which is less than 10% the yield stress of any of the other layers in the element.

2. The photographic element of claim 1 wherein deformable material has plastic deformation stress of 8 MPa and comprises a medium density polyethylene at least 20  $\mu\text{m}$  thick.

3. The photographic element of claim 1 wherein said deformable material comprises medium density polyethylene.

4. The photographic element of claim 1 further comprising an upper sheet of biaxially oriented polymer sheet and a sheet of cellulose paper between said upper sheet and said deformable tie layer material.

5. The photographic element of claim 4 wherein said deformable tie layer material binds said bottom biaxially oriented polymer sheet to said paper.

6. The photographic element of claim 5 wherein said bottom biaxially oriented polymer sheet comprises biaxially oriented polyolefin sheet.

7. The photographic element of claim 5 wherein said base is a polyolefin sheet comprising voids.

8. The photographic element base of claim 4 further comprising a biaxially oriented polyolefin sheet.

9. The photographic element of claim 1 wherein said deformable tie layer material adhesively joins said bottom biaxially oriented polymer sheet to a paper.

10. The photographic element of claim 9 wherein there is a nonvoided polymer layer of said bottom sheet adjacent said cushioning layer.

11. The photographic element of claim 1 wherein said base comprises an upper biaxially oriented polyolefin sheet having at least one voided layer.

\* \* \* \* \*